

## UNITED STATES PATENT OFFICE

2,244,075

## MINERAL OIL PRODUCT

Louis A. Mikeska, Westfield, N. J., assignor to  
 Standard Oil Development Company, a corpora-  
 tion of Delaware

No Drawing. Application October 12, 1938,  
 Serial No. 234,605

9 Claims. (Cl. 252—47)

The present invention relates to improved mineral oil products and more especially to oils, greases and the like which contain addition agents to improve their properties. The invention will be fully understood from the following description.

Many addition agents for lubricating oils or greases have been suggested to improve various properties, especially stability, but few have been found which have the marked advantage in preserving the oils under elevated temperatures, such as are encountered in internal combustion engines and in maintaining a clean engine condition. In the present instance, a new class of chemical substances has been suggested for this purpose and it has been found that these agents are very powerful in reducing carbon formation, the sticking of rings and the deposits in the slits and grooves, and in generally improving engine condition. The particular class referred to above is that of the aromatic sulfenamides and is best described by a structural formula as follows:



where R' and R'' represent hydrocarbon or substituted hydrocarbon groups which will be described more fully below and X represents a hydrogen atom or some other substituent group, more especially nitro groups, amino and hydroxy groups. As indicated above, the benzene ring appearing in the above mentioned formula is preferred, but other aromatic radicals may be employed such as naphthalene, anthracene and phenanthrene rings or their alkylated derivatives. The groups R' and R'' may be hydrocarbon groups, for example alkyl groups such as methyl, ethyl, propyl, butyl or higher alkyl groups and the compounds containing these groups are desirable in reducing the oxidation rate of the oil. In the formula mentioned above R' and R'' are preferably aromatic groups such as phenyl, naphthyl, cresyl, benzyl or various alkylated aromatic groups. Compounds of this type are preferred to those in which R' and R'' are aliphatic because they are particularly desirable and effective in maintaining a clean engine condition. The said aromatic groups may be entirely of a hydrocarbon nature or they may be substituted, that is to say containing elements or radicals with atoms other than hydrogen or carbon. Thus the aromatic groups may be phenolic, containing a free hydroxyl group, or they may be sulfides or disulfides. They may likewise contain nitro or amino groups.

The atom or radical marked X in the above formula is shown in the ortho position for illustration, but it will be understood that the

said group may be in other positions as well or, indeed, if desired no substituent is necessary. The compounds described above may be added to the oil or grease in proportions from about .10 or 1.5 or 2.0%. In this proportion they reduce the corrosive action of oils on alloy bearings such as those composed of copper, lead, cadmium, silver or the like. They likewise reduce the oxidation very markedly and improve the carbon depositing tendency of the oil under high temperature conditions.

The reagents referred to above may be added to oils of all types whether derived from paraffinic, naphthenic or mixed base crudes and may be used either alone or in combination with other well known agents, for example, soaps, heavy metal salts such as naphthenates, or other soluble salts of aluminum, cobalt, nickel, calcium, barium or chromium. They may be used along with dyes, pour point depressants, thickening agents, oiliness or extreme pressure compounds.

## Example I

A lubricating oil of SAE No. 20 was used as a blank and denoted as sample 1. To a sample of this oil was added .25% of di-n-butyl o-nitrobenzene-sulfenamide. This sample was designated sample 2. The formula of the compound added is as follows:



Oxidation rates were determined on the blank and on sample 2 by bubbling oxygen which was passed in a circulatory path including a 10 cc. sample of the oil while held at 200° C. The amount of oxygen absorbed was determined at intervals of 15 minutes by difference from the amount remaining uncombined. The results were as follows:

|          | Oxidation rate |
|----------|----------------|
| Sample 1 | 74—40—35—28    |
| Sample 2 | 15—17—16—14    |

Two samples 1a and 2a, similar to those used above except made up with mineral oil of SAE 40 grade, were then tested for carbon depositing tendency. In this test the oil was slowly dropped into a heated steel cone, having a circumferential groove milled cut in a screw fashion on an inside periphery so as to allow a time of contact of about one minute between the heated surface and the oil. A total volume of 60 cc. of oil is dropped from a dropping funnel during a period of 2 hours to obtain this time of contact. The temperature of the cone may be held at any desired point, but for ordinary testing 250° C. seems preferable because it best approximates

the engine condition. The cone is weighed before the test, and after all the oil is run over the metal surface, it is washed with naphtha to remove the adherent oil and again weighed. The total deposit is obtained by difference in weight. This value is reported in grams of carbon. The following results were obtained:

|           | Cone data,<br>Grams |
|-----------|---------------------|
| Sample 1a | .50                 |
| Sample 2a | .09                 |

It will thus be seen that the addition agent has greatly improved the carbon deposit tendency of this oil.

Sample of coil containing the addition agent was found to be non-corrosive according to the ordinary copper strip test, in spite of the addition of the sulfur in the compound added, and when sample 2 was subjected to the known Underwood test, it was found to be much less corrosive to alloy bearings than was the blank sample 1.

#### Example II

Using the blank oil of Example I, a third sample, No. 3, was made up containing .25% of phenyl-a-naphthyl o-nitrobenzene-sulfenamide:



The oxidation rate of this sample was determined just as in Example I, with the following results:

|          | Oxidation rate |
|----------|----------------|
| Sample 3 | 10-12-13-13    |

It was likewise found to be non-corrosive to the copper strip test.

#### Example III

The addition agent used in Example II was blended in an SAE No. 40 oil and run in a C. F. R. engine for a period of 14 hours. The blank oil (SAE No. 40) containing no addition agent was also run under strictly comparable conditions. After these runs the engines were taken down and the pistons were examined and rated according to their condition. In this examination each part of the piston was examined, for example, the condition of the rings, the ring slits, ring grooves, as well as the total amount of carbon formed, the carbon on the under side of the piston, and the presence or absence of varnish on piston skirt. Separate ratings were given on the basis of these examinations and a composite overall demerit rating was given for the piston. In the following table, this data is summarized:

|                           | Demerits       |                 |                 |            |              |                     |               |               |
|---------------------------|----------------|-----------------|-----------------|------------|--------------|---------------------|---------------|---------------|
|                           | Piston overall | No. rings stuck | Degree sticking | Ring slits | Ring grooves | Carbon under piston | Varnish skirt | Carbon formed |
| Reference oil SAE No. 40  | 4.81           | 3               | 810             | 7.33       | 6.00         | 4.5                 | 5             | Grams 7.35    |
| Ditto + 1/4% of inhibitor | 1.59           | 0               | 0               | 1.00       | 4.00         | 3                   | 4             | 1.80          |

It will be understood that the larger demerit rating indicates a poorer engine condition, and naturally smaller amounts of carbon indicate better performance.

From the test data, it will be seen that the addition of .25% of the reagent has greatly improved the performance of the oil. As a whole, the piston condition is considerably better and in each respect it is also improved. For example, the sticking of rings has been eliminated and the slits and grooves are both improved. The total amount of carbon is greatly diminished and the carbon on the under side of the piston is also diminished. There is likewise less varnish on the skirt. In all, it is clear that the condition of the engine is much better with the oil to which the agent has been added.

The present invention is not to be limited by any theory of the mechanism of the engine improvement or the particular agents, which have been added, but only by the following claims.

I claim:

1. An improved lubricant comprising a hydrocarbon oil and a small amount of an aromatic sulfenamide.
2. An improved lubricant comprising a hydrocarbon oil and a small amount of a compound of the formula:



30 where R' and R'' are hydrocarbon groups.

3. An improved lubricant according to claim 2 in which R' and R'' are aliphatic hydrocarbon radicals.

4. An improved lubricant comprising a hydrocarbon oil and a small amount of a compound of a formula:



45 where R' and R'' are hydrocarbon groups and X is a substituent selected from the class consisting of -NO2, -OH and NH2 groups.

5. An improved lubricant according to claim 4 in which the groups R' and R'' of the added compound are aliphatic.

6. An improved lubricant comprising a mineral lubricating oil and a diaromatic-substituted aromatic sulfenamide.

7. An improved lubricant comprising a mineral lubricating oil and a di-aryl benzene sulfenamide.

8. An improved lubricant comprising a mineral lubricating oil and a di-aryl nitrobenzene sulfenamide.

60 9. An improved lubricant comprising a mineral lubricating oil and a small amount of phenyl-a-naphthyl o-nitrobenzene sulfenamide.